

## UNITED STATES PATENT OFFICE.

ETTA MARIE BURKET, OF BANGOR, MAINE.

## CLEANSING AND POLISHING COMPOUND.

No Drawing. Application filed March 7, 1925. Serial No. 13,913.

*To all whom it may concern:*

Be it known that I, ETTA M. BURKET, a citizen of the United States, residing at Bangor, in the county of Penobscot and State of Maine, have invented certain new and useful Improvements in Cleansing and Polishing Compounds, of which the following is a specification, reference being had to the accompanying drawings.

10 This invention relates to certain improvements in cleansing and polishing compounds and it is an object of the invention to provide a novel and improved compound of this character especially designed and adapted 15 for use in connection with silverware and the like.

It is also an object of the invention to provide a compound of this kind which is in the form of a cake and which is adapted 20 to be applied to the work by a suitable cloth.

My improved compound as herein disclosed comprises the following ingredients: Rouge (jewelers), 2 or 3 teaspoonfuls; white chalk (precipitated), 1 cup; pumice 25 (floated), 1½ cups; warm water, 1 gallon.

After the foregoing ingredients have been thoroughly admixed there is then added 20 pounds of whiting and after continued further mixing the resultant compound is 30 placed in cans or other desired containers and let dry for forty-eight hours, after which the compound is ready for use.

After drying the compound in each of the containers it is substantially in the form of a cake yet can be readily transferred to a suitable cloth upon rubbing such cloth on the cake so that silverware and the like may be effectively cleansed and polished.

The rouge in addition to providing the cleansing and polishing action serves as a binder to maintain the compound in its desired consistency, while the chalk in addition to its polishing action provides a body. The pumice serves as an effective cleansing medium. The whiting also provides an effective polishing medium and also operates as a body and facilitates, owing to the fact that it is last applied, the requisite forming of the cakes.

My improved compound is particularly 50 advantageous for use as it is wholly and entirely non-poisonous nor does it have any aggravating action on the skin whereby the compound may be used without fear of injurious effects of any kind upon the person.

I claim:

A cleansing and polishing compound comprising rouge, precipitated chalk, floated pumice, water, and whiting in the proportions specified.

In testimony whereof I hereunto affix my signature.

ETTA MARIE BURKET.